

July 15, 1924.

1,501,049

A. HARPER

PROCESS FOR PLATING STAINLESS STEEL AND ARTICLES PRODUCED THEREBY

Original Filed Dec. 24, 1921

*Fig. 1.*



*Fig. 2.*



*A. Harper, INVENTOR,  
BY Mitchell & Aecker  
ATTORNEYS*

Patented July 15, 1924.

1,501,049

# UNITED STATES PATENT OFFICE.

ALEXANDER HARPER, OF BRISTOL, CONNECTICUT.

## PROCESS FOR PLATING STAINLESS STEEL AND ARTICLES PRODUCED THEREBY.

Application filed December 24, 1921, Serial No. 524,700. Renewed July 17, 1923.

To all whom it may concern:

Be it known that I, ALEXANDER HARPER, a citizen of the United States of America, residing at Bristol, Connecticut, have invented a new and useful Process for Plating Stainless Steel and Articles Produced Thereby, of which the following is a specification.

My invention relates to a new and improved process for surface finishing articles made of so-called "stainless steel and articles produced thereby." Such articles are described and claimed in the Brearley Patent #1,197,256 dated September 5th, 1916. For the purpose of the present application, I shall describe my process as applied to the finishing of a handle of a steel table knife.

In the accompanying drawing:

Fig. 1 is a side elevation of a table knife, conventionally illustrating the appearance of the handle portion after the article has been subjected to the first step in my process.

Fig. 2 is a similar view of the same article in a finished state, that is to say, after it has been subjected to the final step of the process.

1 represents the polished blade portion of a table knife. 2 represents the handle portion thereof which is formed integrally with the blade. The article is made throughout from so-called "stainless steel" which comprises substantially a ferrous alloy containing between nine per cent (9%) and sixteen per cent (16%) of chromium and carbon in quantity less than seven tenths per cent (.7%), and preferably not containing any microscopically distinguishable free carbids. Otherwise stated, the article is made from a metal alloy such as set forth and claimed in the aforesaid Brearley patent, which article, as is well known, possesses to a remarkable degree the quality of being practically untarnishable, and which articles have so far satisfied that claim that the steel employed in such articles has become widely known as "stainless steel."

Heretofore, it has been regarded as practically impossible to successfully apply to the hardened and polished surfaces of articles made from such steel, a durable electro-plated surface finish. I have found that by subjecting the surface of such articles to the

action of the following acid solution, that said surface may thereby be rendered suitable for receiving and retaining thereon an electro-plate deposit such as silver. In the manufacture of table cutlery, for example table knives, it is highly desirable that the handle portions should be finished with silver even though such handle portion is made of an untarnishable steel. Accordingly, in carrying out my process, I first thoroughly clean the articles and then immerse such portion or portions as it is desired to electro-plate in a solution which contains substantially one part of hydrofluoric acid, six parts nitric acid and thirty-two parts water. I have found that such a solution will attack the otherwise smooth and untarnishable surface in such a manner as to render it relatively rough and make it peculiarly receptive to an electro-plated deposit of silver.

In Fig. 1, I have indicated conventionally and relatively exaggerated, the rough appearance of the handle portion of a table knife after it has been subjected to the action of the aforesaid acid solution. After the article has been thus treated, the surface which has been thus prepared is immersed in an electro-plating bath and subjected to the usual plating treatment, the handle, after such treatment, being represented in Fig. 3. I have found that by this process an entirely satisfactory and commercially successful article can be produced.

While I have described herein the proportions of an acid solution which I know from actual experience will successfully prepare the surface of a "stainless" steel article for electro-plating, it should be understood that this solution may be somewhat changed, the important thing being to provide a solution that will successfully prepare the surface which it is desired to plate by rendering it relatively rough so that the metal deposited thereon will so cling thereto with such tenacity as to successfully resist the uses to which such articles are usually put.

What I claim is:

1. The process of finishing the hardened and smooth surface of an article composed of a ferrous alloy containing between nine per cent (9%) and sixteen per cent (16%) of chromium and carbon in quantity less than seven tenths per cent (.7%) comprising

- ing subjecting the surface of such an article to the action of an acid that will render such surface relatively rough and then depositing a different metal upon such relatively rough surface by an electro-plating process. 5
2. The process of finishing the hardened and smooth surface of a cutlery article composed of a ferrous alloy containing between nine per cent (9%) and sixteen per cent 10 (16%) of chromium and carbon in quantity less than seven tenths per cent (.7%), comprising subjecting the surface of such an article to the action of a solution which will destroy the polish thereon and produce a 15 relatively rough surface and then depositing a different metal upon such relatively rough surface by an electro-plating operation.
3. The process of finishing the hardened 20 and polished surface of a cutlery article composed of a ferrous alloy containing between nine per cent (9%) and sixteen per cent (16%) of chromium and carbon in quantity less than seven tenths 25 per cent (.7%), which comprises subjecting such a portion of the surface as it is desired to finish to the action of an acid solution containing substantially one part hydrofluoric acid, six parts nitric acid and 30 thirty-two parts water until such surface is relatively roughened by the action of such acid and thereafter depositing different metal upon such relatively rough surface by an electro-plating process.
- 35 4. The process of finishing the hardened surface of an article of steel which comprises subjecting such portion of the surface as it is desired to finish to the action of a solution containing substantially one part hydrofluoric acid, six parts nitric acid and thirty-two parts water until such surface is relatively roughened by the action of such solution, and thereafter depositing a 40 different metal upon such relatively rough surface by an electro-plating process.
- 45 5. The process of finishing the surface of an article formed of carbon steel containing chromium and which has been treated to render same relatively non-corrodible by 50 weak acids, comprising subjecting such portion of the surface as it is desired to finish to the action of an acid solution containing hydrofluoric acid until such surface is relatively roughened, and then depositing a dif- 55 ferent metal upon such relatively roughened surface by an electro-plating process.
6. The process of finishing the surface of an article formed of steel containing carbon and chromium and which has been treated to render the same relatively non-corrodible by weak acids, comprising subjecting such portion of the surface of such article as it is desired to finish to the action of an acid that will render such surface relatively rough, and then depositing a different metal upon such relatively rough 60 surface by an electro-plating process. 65
7. The process of finishing the surface of an article formed of carbon steel containing between nine per cent (9%) and sixteen per cent (16%) of chromium, comprising subjecting such portion of the surface of such article as it is desired to finish to the action of an acid that will render such surface relatively rough, and then depositing a different metal upon such relatively rough 70 surface by an electro-plating process. 75
8. As an article of manufacture, an article formed of steel containing carbon and chromium and which is relatively non-corrodible by weak acids, at least a portion of said article being coated with a different metal integrally joined thereto. 80
9. As an article of manufacture, an article formed of carbon steel containing between nine per cent (9%) and sixteen per cent (16%) of chromium, at least a portion of said article being coated with a different metal integrally joined thereto. 85
10. As an article of manufacture, an article of tableware composed of a ferrous alloy containing between nine per cent (9%) and sixteen per cent (16%) of chromium, and carbon in quantity less than seven-tenths per cent (.7%), a portion of said article being coated with a different metal integrally joined thereto. 90 95
11. As an article of manufacture, a knife having integral handle and blade portions formed of a ferrous alloy containing between nine per cent (9%) and sixteen per cent (16%) of chromium, and carbon in quantity less than seven-tenths per cent (.7%), the handle portion of said knife being coated with a different metal integrally joined thereto. 100 105

ALEXANDER HARPER.